

April 24, 1956

H. E. CORBIN ET AL

2,743,179

PITCH CONTROL IN PAPER MAKING

Filed July 22, 1953

3 Sheets-Sheet 1



INVENTORS  
HAROLD E. CORBIN  
JOHN C. DEAN  
BY  
Francis J. Johnston  
AGENT

April 24, 1956

H. E. CORBIN ET AL

2,743,179

PITCH CONTROL IN PAPER MAKING

Filed July 22, 1953

3 Sheets-Sheet 2



INVENTORS  
HAROLD E. CORBIN  
JOHN C. DEAN  
BY *Francis J. Johnston*  
AGENT

April 24, 1956

H. E. CORBIN ET AL

2,743,179

## PITCH CONTROL IN PAPER MAKING

Filed July 22, 1953

3 Sheets-Sheet 3

Fig. 5



BY

INVENTORS  
HAROLD E. CORBIN  
JOHN C. DEAN

Francis F. Johnston

*AGENT*

## 1

2,743,179

## PITCH CONTROL IN PAPER MAKING

Harold Emery Corbin, Arlington, Mass., and John Clark Dean, Port Washington, N. Y., assignors to Socony Mobil Oil Company, Inc., a corporation of New York

Application July 22, 1953, Serial No. 369,608

10 Claims. (Cl. 92—9)

The present invention relates to the control of pitch in paper making and accelerated cooking particularly in the "sulfite" method of pulping.

In general, the efforts exerted in the past to control pitch in paper making have centered around attempts to remove pitch from the machines involved after the pulp is dumped from the digester. It now has been found that pitch can be controlled from its very inception and a much faster cooking operation achieved by introducing a pitch solvent and a non-ionic, an anionic or a cationic emulsifier into the digester.

Pitch is troublesome in paper furnishes containing groundwood and sulfite pulp, particularly when the latter is unbleached. The problem has been considerably aggravated by the use of green-unaged wood which the paper industry has been forced to use in recent years, and which it will continue to use for quite some time.

It has been found that the use of an emulsion of a highly aromatic solvent in the presence of a critical amount of a non-ionic, an anionic or a cationic emulsifier, or in general an emulsifier or dispersing agent effective in acid medium of say pH 5-6, results in:

- (a) A marked decrease in cook cycle,
- (b) A decided improvement in screening conditions and pulp cleanliness,
- (c) Reduction in shut-down time in the Fourdrinier operation and in the operation of the cylinder machines,
- (d) More effective control of slime and bacterial growth and,
- (e) An improved quality pulp.

The efficacy of the pulping agent of the present invention was completely demonstrated on a full plant scale in a pulp mill having eight horizontal indirect cook digesters, each of ten tons finished pulp capacity and charged by a gravity acid system and a small cylinder machine which operates on slush pulp and produces light weight free sheets such as twisting, waxing and carbonizing grades. Operated as a separate unit in conjunction with the pulp mill is a single Fourdrinier paper machine which also manufactures light weight free sheets.

Mill records establish that during test periods of several weeks after continued use of the novel pulping accelerator and pitch dispersant that there was an average increase in tonnage of approximately 25 per cent. This is attributed to a shortened and more uniform cooking cycle and to markedly improved screening conditions. In addition, there was a reduction of slime in the winter months without the use of chemicals for bacteria control while in the warm weather a sizeable reduction of bactericide was possible.

Furthermore, although the actual consumption of chlo-

## 2

rine in bleaching operations has not been noticeably reduced, there has been a noticeable increase in the brightness of the pulp with equivalent amounts of bleaching agent.

Generally, the pitch control and pulp penetrant is added directly to the digester for optimum results either through the acid line feeding into the digester or by other means such as with the wood chips.

When the novel pitch dispersant and cooking accelerator was first added to a digester charge in the mill it was noticed that after about 90 hours of operation at the rate of about an amount of reagent equal to the amount of pitch in the wood being digested, extremely large pitch balls suddenly appeared in the beater furnishing stock to the cylinder machine. This beater was charged with 80 per cent to 90 per cent of unbleached slush pumped directly from the pulp mill and 10 per cent to 20 per cent of bleached laps.

From the dark appearance of the agglomerated material, it was evident that this was pitchy material which had been deposited previously. Close inspection of the screens, the Kaymr cylinder and press section confirmed the foregoing since it was manifest that old deposits of pitch were being removed gradually. In spite of this excessive amount of old pitch, no difficulty was caused in the operation of the Kaymr machine.

Thereafter, the novel reagent was added at the rate of 5 to 10 gallons of reagent per digester charge.

By the use of novel reagent, a quicker cook is achieved. This is clearly shown by the graphs Figures I, II, II and IV. The progress of the cook is determined by measurement of the free sulfur dioxide and the cook is regarded as completed when the sulfur dioxide content drops to 0.2 per cent or less. These data represent several typical periods when the novel reagent was used and when it was not used. In general, the slope of the graphs of cooks without the novel reagent indicate that after a slow initial period the rate of cooking accelerated rapidly after nine hours. On the other hand, when the digestion was carried out in the presence of the novel reagent, the reduction in sulfur dioxide content proceeds more rapidly earlier in the digestion cycle, indicating a definitely quicker cook due to earlier penetration of the wood chips by the digester liquid.

The curves in Figure II derived from data on cooks made without the addition of the novel reagent but after the initial use thereof follow the same pattern as those based upon data obtained while adding the novel reagent and establish the residual effect of the novel reagent.

Operation of this mill, as data for the past several years indicates, involves the devotion of eight to twelve hours every two to three weeks for cleaning the system. Screen capacity being the limiting factor, this has resulted in a production loss of three to five tons of pulp per hour of shutdown time or an average loss of fifty tons per shutdown. It has been established that when the novel reagent is used, the period between shutdowns can be lengthened greatly. During the test period the interval between shutdowns was extended to an average of ten weeks instead of two or three.

As a result of better screening conditions, the amount of tailings is less. The knot rejects from pulp digested in the presence of the novel reagent are softer and contain less entrapped fiber.

In view of the foregoing, it is evident that the present invention provides a means of reducing pitch trouble in sulfite and groundwood pulping mills and involves adding

the novel reagent to the digesters in the sulfite pulping process or to the groundwood in the mechanical process.

The effect of the novel pitch dispersant and pulp penetrant is best recognized from the following interpretation of the records of cook cycle time for the period from November of one year to March of the next succeeding year. Upon the addition of the novel pitch dispersant and pulp penetrant, there was no pronounced fluctuations in cycle time and the cycle time became less until it reached a minimum. The use of the novel reagent was stopped on January 22 according to the pre-arranged plan but the residual effect was apparent until January 28. Thereafter, the time of the cooking cycle increased and became irregular until February 17 when 10 gallons of reagent were added. The effect of the addition of the reagent was not manifest until February 20 when the time of the cycles became less and the fluctuations ceased. This is depicted graphically in Figure V.

In general, the novel pitch dispersant and pulp penetrant comprises a solvent for pitch or resin and non-ionic, anionic or cationic emulsifier. It is preferred to use a high solvent power aromatic oil such as xylene, methyl naphthalenes or, in general, a solvent having a mixed aniline point of 125° F. maximum together with a non-ionic or anionic or cationic emulsifier such as gums, proteins, amines, amine soaps, sulfonates, etc. In order to facilitate the use of the novel reagent, it is also preferred to add the pitch dispersant and pulp penetrant to the pulping system as an emulsion containing 35 per cent to 75 per cent of solvent or base oil and 0.5 per cent to 15.0 per cent of the emulsifier and the balance water. The emulsion so produced is stable in storage and may be subjected to high dilution with water or with acids of the strength customarily used in the sulfite pulping process.

Typical and illustrative of the suitable solvents or base oils are the following cycle oils from a catalytic cracking operation:

| Base Oil.....                  | "A"  | "B"  | "C"  |
|--------------------------------|------|------|------|
| A. P. I. Gravity.....          | 20.8 | 23.6 | 10.0 |
| Flash Point (COC), ° F.....    | 175  | 196  | 260  |
| Pour Point, ° F.....           | 0    | 0    | 0    |
| Viscosity at 100° F. S. U..... | 32.9 | 37   | 37   |
| Mixed Aniline Point, ° F.....  | 88.0 | 97.9 | 59.7 |
| IBP..... ° F.....              | 352  | 416  | 496  |
| 10%.....                       | 404  | 474  | 516  |
| 50%.....                       | 494  | 521  | 536  |
| 90%.....                       | 549  | 596  | 585  |
| FBP.....                       | 600  | 691  | 668  |

Base oil or solvent A comprises primarily mono-substituted alkyl naphthalenes; base oil or solvent C comprises predominantly di-substituted alkyl naphthalenes; and base oil or solvent B comprises mono- and di-substituted alkyl naphthalenes.

Typical of the emulsifiers is the soap formed by the reaction of a carboxylic acid such as acetic acid and a primary aliphatic amine of the type  $RNH_2$  where R is an alkyl radical of 8 to 20 carbon atoms. This cationic emulsifier may be used in the range of 0.75 per cent to 3 per cent amine with the molecular equivalent of the carboxylic acid. Thus, for example, the base oil emulsion may be made by using 1 per cent of  $RNH_2$  and 1 per cent acetic acid as an emulsifier.

The emulsion is most readily and preferably prepared with a minimum amount of emulsifier and a maximum amount of base oil under conditions of high shear in a mechanical homogenizer while maintaining the resultant product in a condition of fluidity. The concentration of the base oil or solvent may vary from 35 per cent to 75 per cent. Thus, for example, a satisfactory pulping adjunct comprised

Solvent ..... percent 70  
Emulsifier ..... do 2  
pH ..... 3.5 to 4.5  
Weight per gal., lbs ..... 7.9

A presently preferred pulping adjunct is one comprising

|                                                    | Weight Percent |           |
|----------------------------------------------------|----------------|-----------|
|                                                    | Broad          | Preferred |
| 5 Solvent <sup>1</sup> .....                       | 40-70          | 60.0      |
| Anionic Dispersing Agent <sup>2</sup> .....        | 0.5-10.0       | 1.2       |
| Protective Colloid <sup>3</sup> .....              | 0.2-2.0        | 0.5       |
| Corrosion Inhibitor <sup>4</sup> .....             | 0.1-2.0        | 0.2       |
| 10 Bactericide and preservative <sup>5</sup> ..... | 0.5-1.0        | 0.1       |
| Formalin <sup>6</sup> .....                        | 0.05-1.0       | 0.1       |
| Water.....                                         | Balance        | 37.9      |

<sup>1</sup> Aromatic petroleum fraction having gravity of 13-17° A. P. I. and boiling range of about 350° to about 600° F.

<sup>2</sup> Alkali metal alkyl aryl sulfonate, sold under trade name of "Marasperse."

<sup>3</sup> Gum ghatti.

<sup>4</sup> Sodium nitrite.

<sup>5</sup> Sodium salt of pentachlorophenol.

<sup>6</sup> Formalin (aqueous 37% formaldehyde).

The essential constituents are the aromatic solvent and the emulsifier or dispersing agent. However, it has been found, particularly when using protective colloids of the nature of organic materials such as gums, that a preservative such as "Dowcide 6," preferably in combination with formalin, are desirable in order to prevent decomposition of the natural organic material of which so many protective colloids such as the natural gums are composed. Sodium nitrite or any other suitable corrosion inhibitor is desirable to inhibit corrosion during storage of the emulsion in metal containers such as shipping containers. Thus, while the essential constituents are the aromatic petroleum fraction or other highly aromatic solvent, the emulsifier, non-ionic, anionic or cationic, and water, it is preferred to incorporate the corrosion inhibitor and the preservative or preservatives in the emulsion.

35 The presently preferred pulping adjunct can be prepared by adding the emulsifiers or dispersing agents "Marasperse N" and Gum ghatti, corrosion inhibitor and high boiling preservative to water with agitation and heating to about 170° F. to complete solution. Thereafter, the solvent is added, the mixture homogenized and cooled to about 110° F. When cooled, the formalin is mixed with the cooled mixture and the pulping adjunct is ready for packaging.

When adding the pulping adjunct to the pulping system, it is preferred to introduce an amount of the adjunct, i. e., 45 emulsion into the pulping system to supply about 0.1 per cent to 1.0 per cent based on the total mass of fibrous materials charged, i. e., wood chips.

This application is a continuation-in-part of our application Serial No. 21,668, filed April 17, 1948.

50 We claim:

1. The improvement in the pulping of wood by the sulfite process which comprises adding to the digester 0.1 to about 1.0 per cent based on total fiber charge to the digester of an emulsion comprising about 35 to about

55 75 per cent of an aromatic petroleum fraction having a mixed aniline point of about 125° F. (maximum), about 0.5 to about 15.0 per cent of an emulsifier effective at pH of about 5 to about 6, and the balance water and digesting said fibre charge in the presence of said emulsion.

2. The improvement in the pulping of wood by the sulfite process which comprises digesting wood chips in the presence of about 2 to about 5 gallons of an emulsion to about ten tons of wood chips, said emulsion

65 comprising about 40 to about 70 weight per cent of an aromatic fraction of mineral oil having an A. P. I. gravity of about 10° to about 24°, a flash point (COC) of about 175° to about 260° F., a viscosity at 100° F. of about 32 to about 37 seconds S. U. V., a mixed aniline point of about 59 to about 98° F., a 10% point of about 400° F. to about 520° F. and a 90% point of about 545° F. to about 585° F., about 0.5 to about 10.0 weight per cent of an anionic emulsifier, about 0.2 to about 2.0 weight per cent of a protective colloid and the balance

70 75 water.

3. The improvement in the pulping of wood by the sulfite process which comprises digesting wood chips in the presence of about 2 to about 5 gallons of an emulsion to about ten tons of wood chips, said emulsion comprising about 40 to about 70 weight per cent of an aromatic fraction of mineral oil having

Gravity °A. P. I., about 10 to about 24

Flash point (COC), about 175° to about 260° F.

S. U. V. @ 100° F., about 32" to about 37"

Mixed aniline pt., about 59° to about 98° F.

10% point, about 400° to about 520° F.

90% point, about 545° to about 585° F.

about 0.5 to about 10 weight per cent of alkali metal lignin sulfonate, about 0.2 to about 2.0 weight per cent Gum Ghatti and the balance water.

4. The improvement in the sulfite pulping of wood which comprises digesting wood chips in the presence of about 0.1 to about 1.0 per cent based upon the total weight of wood chips of an emulsion comprising about 40 to about 70 weight per cent of an aromatic fraction of mineral oil having

Gravity °A. P. I., about 10 to about 24

Flash point (COC), about 175° to about 260° F.

S. U. V. @ 100° F., about 32" to about 37"

Mixed aniline point, about 59° to about 98° F.

10% point, about 400° to about 520° F.

90% point, about 545° to about 585° F.

about 0.5 to about 10 weight per cent of sodium lignin sulfonate, about 0.2 to about 2.0 weight per cent Gum ghatti and the balance water.

5. The improvement in the pulping of wood by the sulfite process which comprises digesting wood chips in the presence of about 0.1 per cent to about 1.0 per cent based on the total mass in the pulping system of an emulsion comprising about 35 per cent to about 75 per cent of an aromatic petroleum fraction having a mixed aniline point of about 125° F. maximum, about 0.5 per cent to about 15.0 per cent of an emulsifier effective in acid medium and the balance water.

6. The improvement in the pulping of wood by the sulfite process which comprises digesting wood chips in the presence of about 2 to about 5 gallons of an emulsion to about ten tons of wood chips, said emulsion comprising about 38 per cent to about 25 per cent of an aromatic fraction of mineral oil having an A. P. I. gravity of about 10° to about 24°, a flash point (COC) of about 175° to about 260° F., a viscosity at 100° F. of about 32 to about 37 seconds S. U. V., a mixed aniline point of about 59 to about 98° F., a 10% point of about 400° to about 520° F. and a 90% point of about 545° to about 585° F., an emulsifier effective in acid medium and the balance water.

7. The improvement in the pulping of wood by the sulfite process which comprises digesting wood chips in the presence of about 2 to about 5 gallons of an emulsion to about 10 tons of wood chips, said emulsion comprising

about 38 per cent to about 25 per cent of a pitch solvent comprising an aromatic petroleum fraction containing primarily alkyl naphthalenes, an emulsifier consisting essentially of about 0.75 to about 3% of a primary aliphatic amine having an alkyl group of 8 to 20 carbon atoms and a molecular equivalent of acetic acid, and the balance water.

8. The improvement in the pulping of wood by the sulfite process which comprises digesting wood pulp in the presence of about 0.1 per cent to about 1.0 per cent based on the total mass in the pulping system of an emulsion comprising about 35 per cent to about 75 per cent of an aromatic petroleum solvent having a gravity of about 10 to about 24° A. P. I., a flash point (COC) of at least about 175° F., a mixed aniline point of about 59° to about 98° F. and a boiling range of about 352° F. to about 691° F., about 0.5 per cent to about 15.0 per cent of an emulsifier consisting essentially of about 0.75 to about 3% of a primary aliphatic amine having an alkyl group of 8 to 20 carbon atoms and a molecular equivalent of acetic acid, an dthe balance water.

9. The improvement in the pulping of wood in the sulfite process which comprises digesting wood chips in the presence of about 2 to about 5 gallons of an emulsion to about 10 tons of wood chips, said emulsion comprising about 35 to about 75 per cent of an aromatic petroleum fraction having a mixed aniline point of about 125° F. maximum and comprising primarily alkyl naphthalenes, an emulsifier consisting of molecular equivalents of a lower aliphatic monocarboxylic acid having not more than 5 carbon atoms and a primary aliphatic amine having an alkyl radical of about 8 to about 20 carbon atoms and the balance water.

10. The improvement in the pulping of wood in the sulfite process which comprises digesting wood chips in the presence of about 2 to about 5 gallons of an emulsifier to about 10 tons of wood chips, said emulsion comprising about 35 per cent to about 75 per cent of an aromatic petroleum fraction having a distillation range of about 200° F. to about 700° F., having a flash point of about 100° F. to about 300° F. and a mixed aniline point of about 59° to about 100° F., an emulsifier consisting essentially of molecular equivalents of acetic acid and a primary aliphatic amine in which the fatty acid radical has about 8 to about 20 carbon atoms.

#### References Cited in the file of this patent

##### UNITED STATES PATENTS

|    |           |             |       |               |
|----|-----------|-------------|-------|---------------|
| 50 | 531,856   | Partington  | ----- | Jan. 1, 1895  |
|    | 1,103,336 | Aktschourin | ----- | July 14, 1914 |
|    | 1,945,862 | McIntyre    | ----- | Feb. 6, 1934  |
|    | 2,144,756 | Fritz       | ----- | Jan. 24, 1939 |

##### FOREIGN PATENTS

|    |         |         |       |                |
|----|---------|---------|-------|----------------|
| 65 | 673,318 | France  | ----- | Jan. 14, 1930  |
|    | 66,695  | Austria | ----- | Sept. 25, 1914 |
|    | 663,444 | Germany | ----- | Aug. 6, 1938   |